

1

3,169,106

HYDROGENATION CATALYST AND PROCESS  
Philip A. Lefrancois, Crawford, Joseph F. McMahon,  
Iselin, and Ernest Solomon, Montclair, N.J., assignors,  
by mesne assignments, to Pullman Incorporated, a cor-  
poration of Delaware  
No Drawing. Filed Aug. 20, 1959, Ser. No. 834,918  
1 Claim. (Cl. 208—111)

This invention relates to a hydrocarbon conversion process involving hydrogen transfer reactions. In one aspect this invention relates to an improved type of catalyst particularly useful for effecting hydrogen transfer reactions and to a method of preparation of such catalyst. In another aspect this invention relates to a process for altering the hydrogen-carbon ratio of a single unsaturated hydrocarbon or mixture of unsaturated hydrocarbons by hydrogenation in the presence of a particular catalyst. In another aspect this invention relates to an improved hydrogenation-hydrocracking process effected in the process of a particular catalyst.

Various types of hydrogen transfer reactions are known to the art including hydrogenation, and hydrocracking or destructive hydrogenation. The treatment of hydrocarbons with hydrogen in the presence of a hydrogenation catalyst is well known in the art. With some exceptions the desirability of liquid fuels and lubricants is roughly proportional to the combined hydrogen that each contains. With the exception of cracked products, however, many petroleum fractions contain little or none of the easily hydrogenated olefinic groups so that deep-seated chemical changes are necessary to promote the entrance of hydrogen atoms into the molecule. High grade kerosenes are made-up of saturated hydrocarbons, paraffins and naphthenes and are low in sulfur, nitrogen and oxygen compounds. However, kerosene distillates from most crudes usually possess few or none of these characteristics. By hydrogenation, aromatics of such kerosene distillates can be converted to naphthenes, any of the paraffins present are saturated while sulfur, nitrogen and other extraneous elements are substantially removed as hydrogen sulfide, ammonia, etc. by the cracking and reduction of corresponding compounds.

The hydrogenation of aromatic hydrocarbons whether they are substantially the only components of the charge stock or are present as components of a hydrocarbon fraction, is relatively difficult to effect. With presently used catalysts, a relatively severe combination of conditions must be applied even with catalysts of high activity. Under such severe conditions the selectivity of catalysis decreases due to concomitant reactions such as hydrocracking. This latter reaction is especially undesirable when it is desired to upgrade a hydrocarbon fraction without substantial change in boiling point, or when it is desired to produce high yields of relatively pure petro-chemicals since it leads to loss of yield of the desired product and makes the process more difficult to control to obtain the desired results.

On the other hand hydrocracking, or destructive hydrogenation, is a process whereby a hydrocarbon fraction is decomposed or cracked to some extent, as well as hydrogenated, in order to make lower boiling products such as, for example, gasoline. It differs from hy-

2

drogenation in that a change in boiling range of a given hydrocarbon fraction is not usually desired in hydrogenation. In addition, hydrocracking is usually effected at a higher temperature and other more severe conditions than normally employed during hydrogenation.

The destructive hydrogenation, hydrocracking or hydrogenolysis of heavy residual hydrocarbon stocks such as reduced crude, vacuum reduced crude, topped crude cracking residuum and like stocks has been known for some time. Useful products, which can be recovered from such a process, include hydrogenated hydrocarbons in the boiling range of gasoline, diesel oil, cycle oil, fuel oil and light gas oil.

Usually, the gasoline boiling range materials are not of exceptional quality and must be subjected to further treatment such as reforming, to provide a good grade of gasoline. Numerous other difficulties have been commonly encountered in the prior art hydrocracking processes, which usually include short catalyst life resulting from excessive carbon deposits on the catalyst surface, low conversion to desired product per pass, and excessive gas formation. In addition, prior art catalysts are susceptible to deactivation by sulfur and other contaminants which are usually present in the feeds employed in hydrocracking processes.

An object of this invention is to provide an improved type of catalyst particularly useful for effecting hydrogen transfer reactions.

Another object of this invention is to provide an improved process for the hydrogenation of aromatic hydrocarbons in good yield and selectivity.

Another object of this invention is to provide a process for hydrogenating a hydrocarbon fraction containing unsaturated hydrocarbons by contacting said fraction with an improved catalyst comprising a compound of molybdenum.

A further object is to provide a new and improved particular hydrogenation catalyst comprising a compound of molybdenum which catalyst is sulfur insensitive and possesses high hydrogenation activity and good thermal stability.

A further object of this invention is to provide an improved hydrocracking process effected in the presence of a particular catalyst of high hydrogenation activity.

It is a further object to provide a method for the preparation of catalysts having the above characteristics. Various other objects and advantages of this invention will become apparent to those skilled in the art from the accompanying description and disclosure.

The above objects are accomplished by providing a catalyst comprising an oxide and/or sulfide of molybdenum and of nickel supported on a silica/alumina support having an alumina content of between about 10 and about 50 weight percent based on the weight of the support. It has been found that the catalysts of this invention possess improved hydrogenation activity as compared with the activity of corresponding catalysts in which an oxide and/or sulfide of cobalt is used in place of the nickel compound, and also possess improved hydrogenation activity as compared with catalysts containing an oxide and/or sulfide of molybdenum and nickel supported on either alumina or silica. It also has been found that the catalysts of this invention are particu-

larly useful as hydrocracking catalysts under appropriate operating conditions.

The content of molybdenum compound (calculated as molybdenum trioxide) in the finished catalyst composite may range between about 3 and about 30 weight percent based on the total weight of the catalyst, and within this range, the concentration of the oxide and/or sulfide of nickel is such to provide an atomic ratio of molybdenum to nickel of between about 1 and about 5. For example, at a concentration of the molybdenum compound within the aforesaid range, the nickel compound is present in an amount between about 0.24 and about 12.2 weight percent (calculated as nickel) based on the total weight of the catalyst. It has been found, however, that superior 10 hydrogenation activity is exhibited by the catalysts in which the oxide and/or sulfide of molybdenum is present in an amount between about 6 and about 20 weight percent at an atomic ratio of molybdenum to nickel of between about 1 and about 3, particularly between about 2 and about 3. The optimum concentration of metal 15 compounds depends to a large extent upon the particular support employed, i.e. on the alumina content of the silica/alumina support, and on the particular reaction to be effected.

Although the support employed for the catalysts of this invention may contain alumina in an amount between about 10 and about 50 weight percent based on the total weight of the support, the preferred catalysts are prepared from silica/alumina supports containing between about 10 and about 30 weight percent alumina. Within an alumina content of between about 10 and about 15 weight percent, optimum activity is observed at a concentration of molybdenum compound of between about 6 and about 12 weight percent, for example, about 8 weight percent, particularly at an atomic ratio of molybdenum to nickel of between about 2 to about 3. On the other hand, when the alumina content is higher, e.g. between about 15 and about 30 weight percent, the optimum content of the molybdenum compound is between about 10 and about 20 weight percent at an atomic ratio of molybdenum to nickel of between about 1 and about 3, particularly between about 2 and about 3.

For the purpose of this invention the support containing between about 10 and about 15 weight percent alumina is referred to herein as the "low" alumina support, and the support containing higher alumina contents, e.g. between about 15 and about 30 weight percent or higher, is referred to herein as the "high" alumina support. This distinction is made since in certain respects, to be more fully discussed hereinafter, catalysts prepared from the low and high alumina supports do not possess the same characteristics or properties.

An alumina content of between about 10 and about 15 weight percent, based on the weight of the support, corresponds to between about 8 and about 14, based on the total weight of the catalyst. Similarly, an alumina content of between about 15 and about 30 weight percent, based on the weight of the support corresponds to between about 11 and about 25 weight percent, based on the total weight of the catalyst.

The silica/alumina support employed in accordance with the teachings of this invention may be prepared by methods well known to those skilled in the art. One method comprises coprecipitation of the oxides or hydrous oxides of aluminum and silicon from aqueous solutions of water soluble salts thereof. Thus, solutions containing appropriate proportions of the water soluble salts of aluminum, such as aluminum chloride, aluminum sulfate, aluminum nitrate and alkali metal aluminates such as sodium aluminate, and of silicon such as the alkali metal silicates, are treated with a basic precipitant, such as ammonium hydroxide, an alkali metal hydroxide or carbonate, or carbon dioxide or acid to precipitate a mixture of the hydrous oxides. The precipitate is then

washed with water to remove water soluble impurities and then dried. Either the water washing or leaching process may be carried out both before and after the drying process. The primary drying operation may be effected at temperatures in the order of 100° F. to 500° F. and then calcined at higher temperatures of between about 750° F. and about 1200° F. Another method comprises commingling an acid such as hydrochloric acid or sulfuric acid with commercial water glass (sodium silicate) under conditions to precipitate silica, washing with acidulated water or otherwise to remove sodium ions, commingling with an aluminum salt such as aluminum chloride and either adding a basic precipitant such as ammonium hydroxide to precipitate alumina, or forming the desired oxide by decomposition of the salt at an elevated temperature as the case permits.

The catalysts of this invention may be prepared by a variety of methods without departing from the scope of this invention. For example, one method comprises impregnating the alumina/silica support with the precursor compound of molybdenum, typical examples of which are silicomolybdcic acid, phosphomolybdcic acid and ammonium molybdate, followed by drying, if desired, and/or calcination at an elevated temperature. The calcined composite is then impregnated with the precursor compound of the nickel compound, typical examples of which are nickel acetate, nickel chloride, nickel sulfate and nickel nitrate, followed by drying, if desired, and/or calcination at an elevated temperature. The reverse order of addition of molybdenum and nickel also leads to active catalysts but generally, when the compounds are added successively, it is preferred to impregnate the silica/alumina support with the molybdenum compound prior to impregnation with the nickel compound. Alternatively, the intermediate calcination step may be omitted. The catalysts of this invention also may be prepared by co-impregnation of the alumina/silica with the molybdenum and nickel precursor compounds. It is to be noted, however, that when co-impregnation is employed, the addition of ammonium hydroxide to the mixture to hold the two compounds in solution has been found to produce a catalyst of lower activity. When the co-impregnation technique is employed, a particularly active catalyst is produced by employing an aqueous solution of phosphomolybdcic acid and nickel acetate.

When employed, the drying steps may be effected at a temperature of between about 100° F. and about 400° F. The intermediate calcination and/or final calcination steps are effected at an elevated temperature such as between about 600° F. and about 1200° F. in the presence of air, nitrogen or other inert gases.

In accordance with a preferred embodiment of this invention, the calcined composite comprising the oxides of molybdenum and nickel is preconditioned with a gaseous stream comprising hydrogen sulfide, or the metal sulfide may be formed in situ such as, for example, when the feed stock to be treated contains a high sulfur content. When the catalysts are preconditioned by contacting with hydrogen sulfide, hydrogen is preferably employed as the carrier gas although other carrier gases such as nitrogen and argon may be employed. The concentration of hydrogen sulfide in the carrier gas may vary between about 0.1 and about 5 mole percent, preferably between about 1 and about 3 mole percent. The preconditioning or activation with hydrogen sulfide may be effected at a temperature between about 400° F. and about 1000° F. and at a pressure between about 50 and about 2000 pounds per square inch gage. As a result of sulfiding, the oxide of molybdenum is converted to a sulfide such as MoS<sub>2</sub> or MoS<sub>3</sub> or mixtures thereof, and the oxide of nickel is converted to a sulfide such as NiS or Ni<sub>2</sub>S<sub>3</sub> or mixtures thereof.

The above-described catalysts find particular utility in the hydrogenation of unsaturated hydrocarbons including olefinsically and aromatically unsaturated compounds.

The feed stock to be hydrogenated may consist of a single unsaturated compound such as when a high purity product is desired or it may comprise a mixture of such hydrocarbons. Thus, for example, aromatically unsaturated compounds such as benzene, toluene, naphthalene, styrene and derivatives thereof are suitable and typical reactants as well as aliphatically unsaturated compounds including acyclic and alicyclic compounds such as, for example, cyclohexene, cyclohexadiene, cyclopentadiene, methylcyclopentene, butenes, pentenes, heptenes, octenes, indene, etc., acetylenes, etc. and mixtures thereof. The process of this invention also may be used to reduce the degree of unsaturation of drying oils.

Also included within the scope of this invention is the hydrogenation of gasoline produced by a catalytic cracking process such gasoline usually being high in olefins, particularly monoolefins. The catalysts of this invention may also be employed to selectively hydrogenate any diolefins which may be present in catalytically cracked gasoline, to convert such diolefins to monoolefins in order to stabilize the gasoline against gum formation. Other feed stocks which may be hydrogenated by the catalysts of this invention are those in which the carbon to hydrogen ratio is high such as reduced crude oil and vacuum tower bottoms, i.e. hydrocarbon stock from which the light fractions have been removed. Hydrogenation of such residual oils increases the gravity thereof and tends to prevent excessive coke laydown during subsequent treatment thereof such as during a subsequent hydrocracking process. In addition, the feed stock may be a hydrocarbon fraction boiling within the range of about 325° F. to about 600° F. such as in particular a kerosene fraction containing unsaturated components. By hydrogenation, the aromatics contained in the petroleum fraction are converted to naphthenes, any of the olefins which may be present are saturated to form a hydrogenated product substantially free of unsaturated components and of improved smoke point. At the same time, sulfur, nitrogen and other extraneous elements which are usually present in the kerosene fraction or vacuum bottom feed stocks, for example, are substantially removed probably in the form of hydrogen sulfide, ammonia, etc.

In accordance with one embodiment of the process of this invention, a hydrocarbon or hydrocarbon fraction is contacted with the catalysts of this invention in the presence of added hydrogen under hydrogenation conditions with net consumption of hydrogen to cause selective hydrogenation of the feed components with minimum hydrocracking to produce product having a lower degree of unsaturation which, in the case of a hydrocarbon fraction boiling within the kerosene range, is evidenced by improvement in smoke point. The hydrogenation process of this invention may be conducted over a wide range of temperatures without departing from the scope of this invention. Such operating conditions include a temperature within the range of from about 200° F. and about 850° F., a pressure between about 0 pound per square inch gage (p.s.i.g.) and about 2000 p.s.i.g. and a space velocity (defined as pounds of feed per hour per pound of catalyst) between about 0.1 and about 10.0. Generally speaking, the conditions within which optimum results are achieved, i.e. high hydrogenation activity and good selectivity, include a temperature of between about 400° F. and about 800° F., a pressure between about 200 and about 800 p.s.i.g. and a weight space velocity of between about 2 and about 10. Hydrogen should be introduced into the reaction zone at a rate of from about 300 to about 20,000 standard cubic feet per barrel (s.c.f.b.) or the hydrogen to hydrogen mole ratio may fall within the range of from about 0.35 to about 50, preferably from about 1 to about 25 moles of hydrogen per mole of hydrocarbon with the total reaction pressure maintained between about 0 and about 2000 pounds per square inch gage (p.s.i.g.), preferably between about 200 and about 800 p.s.i.g. It is desirable that the hydrogen partial pres-

sure be carefully controlled within the preferred range of from about 15 to about 1500 pounds per square inch absolute (p.s.i.a.) preferably from about 100 to about 900 p.s.i.a. to effect the desired conversion while maintaining the activity of the catalyst at a high level.

In accordance with another embodiment of the present invention, a higher boiling hydrocarbon fraction is converted to a lower boiling hydrocarbon fraction by hydrocracking or destructive hydrogenation. That is, in accordance with this embodiment, a hydrocarbon feed stock boiling within the kerosene boiling range and higher is hydrocracked in the presence of added hydrogen or a hydrogen-rich gas, such as re-cycle gas, etc., containing light (C<sub>1</sub>-C<sub>5</sub>) hydrocarbons and under a pressure from about 200 to about 2000 pounds per square inch gage (p.s.i.g.) or higher in contact with the catalysts of this invention. In the hydrogenative cracking zone, or hydrocracking zone, conditions of operation are preferably maintained to favor hydrocracking of the charge without effecting formation of low molecular weight gaseous compounds and little or practically no carbon production such that the process can be operated for comparatively long periods of time before necessitating periodic catalyst regeneration. These conditions include a pressure in the range of from about 200 to about 2000 p.s.i.g., temperatures from about 500 to about 1000° F. and a hydrocarbon space velocity of about 0.1 to about 10 pounds of oil per hour per pound of catalyst with hydrogen being added to the charge or reaction zone at the rate of about 1 to about 50 moles of hydrogen per mole of hydrocarbon feed. In the preferred operation, pressures of about 500 to about 1200 p.s.i.g. are employed, at temperatures of between about 600° F. and about 925° F., and a space velocity of about 0.5 to about 5 with hydrogen being added at rates of about 3 to about 12 moles per mole of hydrocarbon feed. Generally speaking, with any of the presently described catalysts, a less severe combination of temperatures and pressure conditions is employed when the catalysts are used to hydrogenate a feed stock without substantially changing its boiling point, as compared with the combination of operating conditions employed when hydrocracking or change in boiling point of the feed is desired.

Hydrocarbon feeds which may be effectively hydrocracked in the presence of the catalysts of this invention include distillate oils, gas oils, catalytic cracking cycle oils, residual and other heavy petroleum fractions, such as heavy gas oil, residuum from thermal or catalytic cracking processes, petroleum wax fractions, and reduced crudes in general. The term reduced crude as used herein is a crude oil from which the light materials and gasoline boiling range constituents have been removed, and which has then been distilled to remove the gas oils present. The initial boiling point of such an oil is usually about 675° F. to 700° F., although this may vary somewhat. Due to the high hydrogenation activity of the catalysts of this invention, the lower boiling fractions such as gasoline produced by hydrocracking of the heavier or higher boiling feeds, are low in olefins and thus do not necessarily have to be subjected to a subsequent hydrogenation treatment prior to use.

The catalysts of this invention are also useful for desulfurizing hydrocarbon oils, e.g. naphthas, kerosene, gasoline, gas oils, total crudes, etc. The desulfurization is effected at a temperature of about 600° F. to about 900° F., preferably about 650° F. to about 850° F. The desulfurization reactions can be effected at either exceptionally high pressures in the order of up to about 2000 p.s.i.g. or at pressures as low as 100 p.s.i.g. More usually, desulfurization by means of the catalysts of this invention is accomplished at a pressure of about 500 to about 1000 p.s.i.g. The desulfurization is effected in the presence of hydrogen and the conditions of operation are such that hydrogen is consumed in the operation. Generally, the hydrogen is supplied to the process at the

rate of about 1000 to about 20,000 s.c.f.b., preferably at a rate of between about 3000 and about 10,000 s.c.f.b. Generally, the weight space velocity ranges between about 0.1 and about 15 pounds per hour of hydrocarbon feed charged to the desulfurization zone per pound of catalyst present therein, and more usually from about 3 to about 8. It is to be understood that hydrodesulfurization also may occur during the above-described hydrogenation or hydrocracking processes.

The catalysts of this invention may be employed effectively as pellets, pills, spheres, rings, extrusions, lumps, granules, extrusions or in a powdered state and these forms may be used in both fluidized systems and those employing moving beds of contact material in either concurrent or countercurrent flow relative to the reactants. The catalysts may also be employed in a slurry type system without departing from the scope of this invention.

The following examples are offered as a better under-

Catalysts I through VIII and Catalysts XIII through XV were prepared from the same fresh "low" alumina/silica cracking catalysts containing 13 weight percent alumina and 87 weight percent silica. As may be seen from Table I, the molybdenum oxide concentration of Catalysts I through VIII ranged between about 3 and about 30 weight percent based on the total weight of the catalyst, the corresponding alumina content ranging between about 13 and about 9 weight percent, based on the total weight of the catalyst.

The support employed in the preparation of Catalysts IX through XII was the same fresh "high" alumina/silica cracking catalyst containing 25 weight percent alumina and 75 weight percent silica. As may be seen from Table I, the molybdenum oxide content ranged between about 3 and about 30 weight percent, the corresponding alumina content ranging between about 24 and about 16 weight percent, based on the total weight of the catalyst.

TABLE I  
*Preparation of Catalysts I-XV*

| Catalyst No. | Weight of Support (grams) | Ammonium Molybdate, grams in H <sub>2</sub> O (cc.) | Dried at 250° F. (hours) | Nickel Acetate, grams in H <sub>2</sub> O (cc.) | Dried at 250° F. (hours) | Composition <sup>4</sup> (weight percent based on total weight of catalyst) |      |                                |                  |       |       |
|--------------|---------------------------|-----------------------------------------------------|--------------------------|-------------------------------------------------|--------------------------|-----------------------------------------------------------------------------|------|--------------------------------|------------------|-------|-------|
|              |                           |                                                     |                          |                                                 |                          | MoO <sub>3</sub>                                                            | NiO  | Al <sub>2</sub> O <sub>3</sub> | SiO <sub>2</sub> |       |       |
| I            | 1 96.36                   | 3.70                                                | 75                       | 20                                              | 1.72                     | 80                                                                          | 21   | 3.02                           | 0.62             | 12.52 | 84.8  |
| II           | 1 46.36                   | 3.70                                                | 45                       | 26.5                                            | 1.74                     | 35                                                                          | 26   | 6.04                           | 1.24             | 12.06 | 80.65 |
| III          | 1 454.50                  | 46.29                                               | 450                      | 15.5                                            | 21.94                    | 500                                                                         | 19   | 7.55                           | 1.55             | 11.82 | 79.07 |
| IV           | 1 43.93                   | 6.17                                                | 45                       | 26                                              | 2.97                     | 35                                                                          | 25.5 | 10.07                          | 2.07             | 11.42 | 76.44 |
| V            | 1 40.90                   | 9.26                                                | 45                       | 21.5                                            | 4.46                     | 35                                                                          | 20   | 15.10                          | 3.10             | 10.63 | 71.18 |
| VI           | 1 23.16                   | 5.51                                                | 35                       | 16                                              | 7.58                     | 30                                                                          | 21.5 | 15.0                           | 7.79             | 10.04 | 67.14 |
| VII          | 1 25.03                   | 5.51                                                | 35                       | 18.5                                            | 1.51                     | 30                                                                          | 23   | 15.0                           | 1.5              | 10.85 | 72.6  |
| VIII         | 1 31.76                   | 18.51                                               | 45                       | 22                                              | 9.13                     | 45                                                                          | 22.5 | 30.2                           | 6.27             | 9.0   | 60.6  |
| IX           | 2 3 24.09                 | 0.92                                                | 20                       | 25.5                                            | 0.51                     | 20                                                                          | 23.5 | 3.02                           | 0.63             | 24.1  | 72.3  |
| X            | 2 3 22.73                 | 2.31                                                | 20                       | 24.5                                            | 1.26                     | 20                                                                          | 21.6 | 7.55                           | 1.55             | 22.7  | 68.2  |
| XI           | 2 3 20.45                 | 4.63                                                | 20                       | 24                                              | 2.51                     | 20                                                                          | 23.5 | 15.1                           | 3.1              | 20.4  | 61.4  |
| XII          | 2 31.76                   | 18.51                                               | 100                      | 21                                              | 9.47                     | 100                                                                         | 17.5 | 30.2                           | 6.42             | 15.83 | 47.49 |
|              |                           |                                                     |                          |                                                 | Cobalt Acetate           |                                                                             |      |                                |                  |       |       |
| XIII         | 1 24.19                   | 0.91                                                | 25                       | 16.3                                            | 0.58                     | 25                                                                          | 25.5 | 3.02                           | 0.6              | 12.5  | 83.9  |
| XIV          | 1 22.74                   | 2.29                                                | 25                       | 24.5                                            | 1.46                     | 25                                                                          | 20   | 7.55                           | 1.55             | 11.81 | 79.1  |
| XV           | 1 24.56                   | 5.51                                                | 35                       | 18.5                                            | 3.56                     | 30                                                                          | 23.5 | 15.0                           | 3.1              | 10.6  | 71.2  |

<sup>1</sup> Support used contained 13 weight percent alumina and 87 weight percent silica.

<sup>1</sup> Support used contained 13 weight percent alumina and 87 weight percent silica.  
<sup>2</sup> Support used contained 25 weight percent alumina and 75 weight percent silica.

3 Support was calcined 1 hour at 1000° F. prior to impregnation.

<sup>4</sup> Calculated, based upon ingredients employed in preparing the catalyst.

standing of the present invention and are not to be construed as unnecessarily limiting thereto.

Catalysts I through XII containing molybdenum oxide and nickel oxide, and Catalysts XIII through XV containing molybdenum oxide and cobalt oxide, on an alumina/silica support, were prepared by the following general procedure: In each instance the alumina/silica support was impregnated with an aqueous solution of ammonium molybdate tetrahydrate  $(\text{NH}_4)_6\text{Mo}_7\text{O}_{24} \cdot 4\text{H}_2\text{O}$ . The impregnated support was then placed in an oven and dried at 250° F., and the dried composite was then ground to a powder and calcined at 1000° F. for 2 hours. In preparing Catalysts I through XII the calcined material thus prepared was impregnated with an aqueous solution of nickel acetate tetrahydrate. In the preparation of Catalysts XIII through XV the calcined impregnated silica/alumina support was impregnated with an aqueous solution of cobalt nitrate hexahydrate instead of nickel acetate. In each instance the mixtures were stirred thoroughly and then dried in an oven at 250° F., ground to a powder and then calcined for 2 hours at 1000° F. The details of these preparations are set forth in the following Table I in which the calculated chemical composition of the final catalyst, based upon the amount of ingredients employed in the preparation of the catalyst, also is given. The atom ratio of Mo/Ni of each of Catalysts I through V and VIII through XII was 2.5, while that of Catalysts VI and VII were 1 and 5, respectively.

HYDROGENATION RUNS

The relative effectiveness of each of the above-described catalysts to effect hydrogenation was determined by using the same in a laboratory hydrogenation test unit using benzene as a typical test feed, the test operation being carried out at conversions well below equilibrium conditions in order to obtain an accurate comparison of the catalyst activities. In these tests, the reactor (8" long with 1/2" inner diameter) was charged with 1 to 5 grams of catalyst powder using glass wool as packing, and alundum as the preheat zone. The reactor was connected into the unit and a hydrogen-hydrogen sulfide gas mixture containing 2 mole percent hydrogen sulfide was passed through the reactor at a pressure of between about 310 and about 330 p.s.i.g. The temperature was then raised to about 750° F., and the reactor was held under these conditions for 1 to 1.5 hours while passing the  $H_2/H_2S$  gas stream therethrough. At the start of each run, the  $H_2/H_2S$  stream was then allowed to pick up benzene, the mole percent of benzene in the  $H_2/H_2S$  stream being constant at 0.55. In testing each catalyst the flow rate of the  $H_2/H_2S$  benzene mixture through the reactor was changed in order to obtain at least two different conversions for each catalyst in order to obtain a sufficient number of conversion values for calculation of the hydrogenation rate constant at a definite tempera-

ture, i.e. at 750° F. expressed as  $k_{750}$ ° F. The value of "k" represents the efficiency of the catalyst to hydrogenate benzene to saturated liquid product at standard conditions of about 325 p.s.i.g. and 750° F. in the above-described system, and it relates to space velocity and conversion. The "k" value was then converted to the space velocity required to obtain a 90 percent conversion of benzene under these test conditions. It should be borne in mind that in this test operation the contact time in each instance was very low due to the fact that only a small quantity of catalyst was employed. This was done in order to operate well below equilibrium conditions and thus obtain accurate comparisons. In each instance, however, at higher contact times, i.e. in the presence of more catalyst, the conversion of benzene in each instance is proportionately higher, but the activity of the catalyst remains the same. The specific test conditions employed and results of these runs are set forth in the following Table II.

TABLE II  
Hydrogenation of benzene

| Run No.                                                     | 1      | 2      | 3   | 4      | 5      | 6      |
|-------------------------------------------------------------|--------|--------|-----|--------|--------|--------|
| Catalyst No.                                                | I      | XIII   | III | XIV    | V      | XV     |
| Composition:                                                |        |        |     |        |        |        |
| Percent MoO <sub>3</sub>                                    | 3.0    | 3.0    | 7.6 | 7.6    | 15.1   | 15.1   |
| Percent NiO                                                 | 0.6    |        | 1.6 |        | 3.1    |        |
| Percent CoO                                                 |        | 0.6    |     |        |        |        |
| Support                                                     | (1)    | (1)    | (1) | (1)    | (1)    | (1)    |
| Pretreatment of Catalyst:                                   |        |        |     |        |        |        |
| Catalyst charge, grams                                      | 1.0    | 1.0    | 1.0 | 1.0    | 2.0    | 5.0    |
| Catalyst Temperature, ° F.                                  | 750    | 750    | 750 | 750    | 750    | 750    |
| Reaction Pressure, p.s.i.g.                                 | 324    | 325    | 325 | 325    | 313    | 329    |
| Gas Composition                                             | (2)    | (2)    | (2) | (2)    | (2)    | (2)    |
| Treatment time, hours                                       | 1      | 1      | 1   | 1      | 1.0    | 1.5    |
| Test Conditions:                                            |        |        |     |        |        |        |
| Catalyst Temperature, ° F.                                  | 750    | 750    | 750 | 750    | 750    | 750    |
| Reaction Pressure, p.s.i.g.                                 | 324    | 325    | 325 | 325    | 314    | 335    |
| Flow rate, standard cc/min                                  | 63     | 90     | 80  | 82     | 80     | 103    |
| Feed                                                        | (3)    | (3)    | (3) | (3)    | (3)    | (3)    |
| Carrier Gas                                                 |        |        |     |        |        |        |
| Results:                                                    |        |        |     |        |        |        |
| Conversion, percent                                         | 19.9   | 15.5   | 0.3 | 5.9    | 24.6   | 32.2   |
| Hydrogenation activity constant $k_{750}$ ° F.              | 14.2   |        | 7.8 |        | 37.5   | 45     |
| Space velocity required to obtain 90% conversion of benzene | 0.0084 | 0.0019 |     | 0.0089 | 0.0034 | 0.0085 |

<sup>1</sup> 13 weight percent alumina/silica. <sup>2</sup> 2 mole percent H<sub>2</sub>S in H<sub>2</sub>. <sup>3</sup> Benzene.

From the data of Table II, it is apparent that the catalysts of this invention containing compounds of nickel and molybdenum on alumina/silica possess significantly higher hydrogenation activity than the catalysts containing compounds of cobalt and molybdenum on the same support at substantially the same concentration of such compounds as tested under substantially the same operating conditions. The superiority of the nickel-containing catalysts is particularly marked at concentrations of molybdenum oxide of at least 7.6 as seen by comparison of the activity constant of Catalysts III and XIV employed in runs 3 and 4, respectively, and of Catalysts V and XV employed in runs 5 and 6, respectively. It is also noteworthy that when the concentration of molybdenum compound is increased in the cobalt-containing catalyst from 7.6 (Catalyst XIV) to 15.1 (Catalyst XV), the activity of the catalyst decreases about 44 percent whereas the same increase of the molybdenum concentration of the nickel catalyst lowered the activity of the catalyst by only about 4 percent. This latter comparison is significant from the standpoint of demonstrating that the molybdenum-nickel catalysts are basically different

compositions from the molybdenum-cobalt compositions.

The improved activity of the catalysts of this invention also is demonstrated by comparing their hydrogenation activity with the activity of catalysts containing approximately the same level of molybdenum oxide and nickel oxide content supported on adsorptive alumina carriers and silica as typically represented by Catalysts XVI, XVII and XVIII, which were prepared as follows:

#### CATALYST XVI

A solution of 3.46 grams of phosphomolybdic acid hydrate, H<sub>3</sub>PMo<sub>12</sub>O<sub>40</sub>·H<sub>2</sub>O (72.69% MoO<sub>3</sub>), and 1.72 grams of nickel acetate tetrahydrate dissolved in 30 cc. of distilled water was added to 21.96 grams of gamma-alumina analyzing 99 percent Al<sub>2</sub>O<sub>3</sub>, 0.02 percent SiO<sub>2</sub>, 0.06 percent Na<sub>2</sub>O and 0.03 percent Fe<sub>2</sub>O<sub>3</sub>. After the mixture was stirred thoroughly, the excess water was removed by evaporation. The mixture was then dried at

10

15

75

210° F. for 22 hours, ground to a powder and then calcined for 2 hours at 1000° F. The calculated composition

55 of the finished catalyst, based upon ingredients, is 10.07 weight percent MoO<sub>3</sub>, 2.07 weight percent NiO,

0.53 weight percent H<sub>3</sub>PO<sub>4</sub> and 87.1 weight percent Al<sub>2</sub>O<sub>3</sub>,

the Mo/Ni atom ratio being 2.5.

#### CATALYST XVII

A solution of 3.46 grams of phosphomolybdic acid hydrate, H<sub>3</sub>PMo<sub>12</sub>O<sub>40</sub>·H<sub>2</sub>O (72.69% MoO<sub>3</sub>), and 1.72 grams of nickel acetate tetrahydrate dissolved in 30 cc. of distilled water was added to 21.96 grams of eta-alumina analyzing 99.8 weight percent Al<sub>2</sub>O<sub>3</sub>. After the mixture was stirred thoroughly, the excess water was removed by evaporation. The mixture was then dried at 210° F. for about 18 hours, ground to a powder and then calcined for 2 hours at 1000° F. The calculated composition of the finished catalyst, based upon ingredients, is 10.07 weight percent MoO<sub>3</sub>, 2.07 weight percent NiO, 0.53 weight percent H<sub>3</sub>PO<sub>4</sub> and 86.15 weight percent Al<sub>2</sub>O<sub>3</sub>, the Mo/Ni atom ratio being 2.5.

60

65

70

## CATALYST XVIII

To 18.5 grams of desiccant grade silica gel (99.9 weight percent  $\text{SiO}_2$ ) which had been calcined for 2 hours at 1000° F. there was added a solution of 1.4 grams of ammonium molybdate tetrahydrate in 10 cc. of distilled water. The paste was mixed thoroughly and then dried in an oven at 250° F. for 18 hours. To the dried solid there was then added an additional amount of aqueous solution of ammonium molybdate tetrahydrate solution, 10 0.824 gram of  $(\text{NH}_4)_6\text{Mo}_7\text{O}_{24} \cdot 2\text{H}_2\text{O}$  in water to wet the solid thoroughly. This mixture was then dried in an oven at 250° F. for about 18 hours, followed by calcination for 2 hours at 1000° F. The calcined composite (20.16 grams) was then impregnated with an aqueous solution containing 1.27 grams of nickel acetate tetrahydrate to give a homogeneous paste which was then dried at 250° F., followed by calcination for 2 hours at 1000° F. The calculated composition, based upon ingredients, was 9.01 weight percent  $\text{MoO}_3$ , 1.87 weight percent  $\text{NiO}$  and 89.1 weight percent  $\text{SiO}_2$ , the Mo/Ni atom ratio being 2.5.

Catalysts XVI, XVII and XVIII were tested as hydrogenation catalysts using substantially the same test procedure and operating conditions employed in carrying out the above-described runs 1 through 6 of Table II. The specific operating conditions and results obtained are set forth in the following Table III which also sets forth, for the purpose of comparison, the results obtained with the above-described Catalysts IV and X which were prepared from the "low" and "high" alumina/silica supports, respectively.

TABLE III  
Hydrogenation of benzene

| Run No.                                                     | 7             |     | 8           |     | 9      |     | 10                 |      | 11                 |      |
|-------------------------------------------------------------|---------------|-----|-------------|-----|--------|-----|--------------------|------|--------------------|------|
|                                                             | XVI           |     | XVII        |     | XVIII  |     | IV                 |      | X                  |      |
| Catalyst No.                                                |               |     |             |     |        |     |                    |      |                    |      |
| Composition:                                                |               |     |             |     |        |     |                    |      |                    |      |
| Percent $\text{MoO}_3$                                      | 10.1          |     | 10.1        |     | 9.0    |     | 10.1               |      | 7.6                |      |
| Percent $\text{NiO}$                                        | 2.1           |     | 2.1         |     | 1.9    |     | 2.1                |      | 1.6                |      |
| Support:                                                    | Gamma-alumina |     | Eta-alumina |     | Silica |     | 13% alumina/silica |      | 25% alumina/silica |      |
| Pre-treatment of Catalyst:                                  |               |     |             |     |        |     |                    |      |                    |      |
| Catalyst charge, grams                                      | 1.0           |     | 1.0         |     | 5.0    |     | 1.0                |      | 1.0                |      |
| Catalyst Temperature, °F.                                   | 750           |     | 750         |     | 750    |     | 750                |      | 750                |      |
| Reaction Pressure, p.s.i.g.                                 | 325           |     | 325         |     | 330    |     | 325                |      | 325                |      |
| Gas Composition                                             | (1)           |     | (1)         |     | (1)    |     | (1)                |      | (1)                |      |
| Treatment time, hours                                       | 1             |     | 1           |     | 1.5    |     | 1                  |      | 1                  |      |
| Test Conditions:                                            |               |     |             |     |        |     |                    |      |                    |      |
| Catalyst Temperature, °F.                                   | 750           |     | 750         |     | 750    |     | 750                |      | 750                |      |
| Reaction Pressure, p.s.i.g.                                 | 325           |     | 325         |     | 322    |     | 325                |      | 325                |      |
| Flow rate, standard cc./min.                                | 113           | 81  | 43          | 108 | 61     | 298 | 131                | 261  | 161                | 120  |
| Feed                                                        | (2)           | (2) | (2)         | (2) | (2)    | (2) | (2)                | (2)  | (2)                | (2)  |
| Carrier Gas                                                 | (1)           | (1) | (1)         | (1) | (1)    | (1) | (1)                | (1)  | (1)                | (1)  |
| Results:                                                    |               |     |             |     |        |     |                    |      |                    |      |
| Conversion, percent                                         | 6.0           | 7.8 | 9.0         | 8.2 | 14.0   | 11  | 13                 | 20.4 | 21.7               | 30.2 |
| Hydrogenation activity constant $k_{H_2O}^{\text{mo}}$      | 6.5           |     | 9.1         |     | 4.6    |     | 54.7               |      | 45.5               |      |
| Space velocity required to obtain 90% conversion of benzene | 0.0015        |     | 0.0022      |     | 0.0011 |     | 0.0130             |      | 0.0108             |      |

<sup>1</sup> 2 mole percent  $\text{H}_2\text{S}$  in  $\text{H}_2$ . <sup>2</sup> Benzene.

From the data of Table III above, it may be seen that the catalysts of this invention, e.g. Catalyst IV employed in run No. 10, and Catalyst X employed in run No. 11, possessed outstanding activity for the hydrogenation of benzene as compared with the alumina-supported Catalysts XVI and XVII, employed in runs 7 and 8, respectively, and the silica-supported Catalyst XVIII, employed in run 9.

The above Catalysts V, VI and VII, prepared as described in Table I above, were tested under the conditions set forth in the following Table IV using substantially the same test procedure described above in carrying out the runs of Tables II and III. These runs were made in order to test the effect of varying the atom ratio of Mo/Ni at a constant concentration of molybdenum oxide. That is, each of these catalysts contained 15.1 weight percent  $\text{MoO}_3$  with varying amounts of  $\text{NiO}$  to provide Mo/Ni

atom ratios of 1 (Catalyst VI), 2.5 (Catalyst V) and 5 (Catalyst VII). The specific operating conditions and results of these runs are given in the following Table IV.

5

## 12

ratios of 1 (Catalyst VI), 2.5 (Catalyst V) and 5 (Catalyst VII). The specific operating conditions and results of these runs are given in the following Table IV.

15

## TABLE IV

## Hydrogenation of benzene

| Run No.                                                     | 12           |      | 13     |     | 14     |      |
|-------------------------------------------------------------|--------------|------|--------|-----|--------|------|
|                                                             | Catalyst No. | VI   | V      | VII |        |      |
| Composition:                                                |              |      |        |     |        |      |
| Percent $\text{MoO}_3$                                      | 15.0         |      | 15.1   |     | 15.0   |      |
| Percent $\text{NiO}$                                        | 7.8          |      | 3.1    |     | 1.5    |      |
| Mo/Ni atom ratio                                            | 1            |      | 2.5    |     | 5      |      |
| Support                                                     | (1)          |      | (1)    |     | (1)    |      |
| Pre-treatment of Catalyst:                                  |              |      |        |     |        |      |
| Catalyst charge, grams                                      | 5.0          |      | 2.0    |     | 5.0    |      |
| Catalyst Temperature, °F.                                   | 750          |      | 750    |     | 750    |      |
| Reaction Pressure, p.s.i.g.                                 | 320          |      | 313    |     | 321    |      |
| Gas Composition                                             | (2)          |      | (2)    |     | (2)    |      |
| Treatment time, hours                                       | 1.0          |      | 1.0    |     | 1.0    |      |
| Test Conditions:                                            |              |      |        |     |        |      |
| Catalyst Temperature, °F.                                   | 750          |      | 750    |     | 750    |      |
| Reaction Pressure, p.s.i.g.                                 | 320          |      | 314    |     | 321    |      |
| Flow rate, standard cc./min.                                | 174          | 235  | 137    | 75  | 119    | 157  |
| Feed                                                        | (2)          | (2)  | (2)    | (2) | (2)    | (2)  |
| Carrier Gas                                                 | (2)          | (2)  | (2)    | (2) | (2)    | (2)  |
| Results:                                                    |              |      |        |     |        |      |
| Conversion, percent                                         | 61.5         | 48.4 | 45     | 56  | 60.2   | 45.7 |
| Hydrogenation activity constant $k_{H_2O}^{\text{mo}}$      | 32.5         |      | 36     |     | 20.8   |      |
| Space velocity required to obtain 90% conversion of benzene | 0.0077       |      | 0.0085 |     | 0.0049 |      |

<sup>1</sup> 13 weight percent alumina/silica.

<sup>2</sup> 2 mole percent  $\text{H}_2\text{S}$  in  $\text{H}_2$ .

<sup>3</sup> Benzene.

30

25

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

30

TABLE V

## Hydrogenation of benzene

| Run No.                                                     | 15               | 16               | 17               | 18               | 19               |
|-------------------------------------------------------------|------------------|------------------|------------------|------------------|------------------|
| Catalyst No.                                                | I                | IX               | II               | III              | X                |
| Composition:                                                |                  |                  |                  |                  |                  |
| Percent MoO <sub>3</sub>                                    | 3.0              | 3.0              | 6.0              | 7.6              | 7.6              |
| Percent NiO                                                 | 0.6              | 0.6              | 1.2              | 1.6              | 1.6              |
| Alumina/Silica Support, Weight Percent                      |                  |                  |                  |                  |                  |
| Alumina, based on support                                   | 13               | 25               | 13               | 13               | 25               |
| Pretreatment of Catalyst:                                   |                  |                  |                  |                  |                  |
| Catalyst charge, grams                                      | 1.0              | 1.0              | 2.0              | 1.0              | 1.0              |
| Catalyst Temperature, ° F                                   | 750              | 750              | 750              | 750              | 750              |
| Reaction Pressure, p.s.i.g.                                 | 324              | 325              | 330              | 325              | 325              |
| Gas Composition                                             | ( <sup>1</sup> ) | ( <sup>1</sup> ) | ( <sup>1</sup> ) | ( <sup>1</sup> ) | ( <sup>1</sup> ) |
| Treatment time, hours                                       | 1.0              | 1.0              | 1.0              | 1.0              | 1.0              |
| Test Conditions:                                            |                  |                  |                  |                  |                  |
| Catalyst Temperature, ° F                                   | 750              | 750              | 750              | 750              | 750              |
| Reaction Pressure, p.s.i.g.                                 | 324              | 325              | 334              | 325              | 325              |
| Flow rate, standard cc./min.                                | 63               | 90               | 112              | 163              | 120              |
| Feed                                                        | ( <sup>2</sup> ) | ( <sup>2</sup> ) | ( <sup>2</sup> ) | ( <sup>2</sup> ) | ( <sup>2</sup> ) |
| Carrier Gas                                                 | ( <sup>1</sup> ) | ( <sup>1</sup> ) | ( <sup>1</sup> ) | ( <sup>1</sup> ) | ( <sup>1</sup> ) |
| Results:                                                    |                  |                  |                  |                  |                  |
| Conversion, percent                                         | 19.9             | 15.5             | 17.3             | 12.9             | 27.7             |
| Hydrogenation activity constant $k_{750^{\circ} F}$         | 14.2             | 22.2             | 24.6             | 31.8             | 34.8             |
| Space velocity required to obtain 90% conversion of benzene | 0.0034           | 0.0053           | 0.0043           | 0.0089           | 0.0108           |

| Run No.                                             | 20               | 21               | 22               | 23               | 24               |
|-----------------------------------------------------|------------------|------------------|------------------|------------------|------------------|
| Catalyst No.                                        | IV               | V                | XI               | VIII             | XII              |
| Composition:                                        |                  |                  |                  |                  |                  |
| Percent MoO <sub>3</sub>                            | 10.1             | 15.1             | 15.1             | 30.2             | 30.2             |
| Percent NiO                                         | 2.1              | 3.1              | 3.1              | 6.3              | 6.4              |
| Alumina/Silica Support, Weight percent              |                  |                  |                  |                  |                  |
| Alumina, based on support                           | 13               | 13               | 25               | 13               | 25               |
| Pretreatment of Catalyst:                           |                  |                  |                  |                  |                  |
| Catalyst charge, grams                              | 1.0              | 2.0              | 1.0              | 5.0              | 5.0              |
| Catalyst Temperature, ° F                           | 750              | 750              | 750              | 750              | 750              |
| Reaction Pressure, p.s.i.g.                         | 325              | 313              | 325              | 320              | 330              |
| Gas Composition                                     | ( <sup>1</sup> ) | ( <sup>1</sup> ) | ( <sup>1</sup> ) | ( <sup>1</sup> ) | ( <sup>1</sup> ) |
| Treatment time, hours                               | 1.0              | 1.0              | 1.0              | 1.0              | 1.0              |
| Test Conditions:                                    |                  |                  |                  |                  |                  |
| Catalyst Temperature, ° F                           | 750              | 750              | 750              | 750              | 750              |
| Reaction Pressure, p.s.i.g.                         | 325              | 314              | 325              | 320              | 330              |
| Flow rate, standard cc./min.                        | 161              | 218              | 261              | 150              | 144              |
| Feed                                                | ( <sup>2</sup> ) | ( <sup>2</sup> ) | ( <sup>2</sup> ) | ( <sup>2</sup> ) | ( <sup>2</sup> ) |
| Carrier Gas                                         | ( <sup>1</sup> ) | ( <sup>1</sup> ) | ( <sup>1</sup> ) | ( <sup>1</sup> ) | ( <sup>1</sup> ) |
| Results:                                            |                  |                  |                  |                  |                  |
| Conversion, percent                                 | 30.2             | 21.7             | 20.4             | 45               | 62.3             |
| Hydrogenation activity constant $k_{750^{\circ} F}$ | 54.7             | 20.4             | 45               | 35.6             | 55.4             |
| Space velocity required to obtain 90% conversion    | 0.1030           | 0.0085           | 0.0153           | 0.0046           | 0.0066           |

<sup>1</sup> 2 mole percent H<sub>2</sub>S in H<sub>2</sub>. <sup>2</sup> Benzene.

From the data of Table V, it is apparent that the catalysts of this invention, and particularly Catalysts III, IV, V, X, and XI, containing above 6 and less than 30 weight percent molybdenum oxide, exhibit outstanding hydrogenation activity. Generally speaking, at the same level of concentration of molybdenum and nickel catalytic agents, the catalysts prepared from the alumina/silica support containing 25 weight percent alumina exhibit higher hydrogenation activity than those prepared from the support containing about 13 weight percent alumina, the highest hydrogenation activity being exhibited by Catalyst XI.

In each of the runs of Table V above, the support was a fresh alumina/silica support having a relative cracking activity of about 1.5. In order to test the effect of employing a support which has previously been de-surfaced by treatment with steam at an elevated temperature, another series of catalysts, i.e. Catalysts XIX to XXX, was prepared using de-surfaced supports. Catalysts XIX to XXX were prepared using substantially the same procedure employed to prepare the catalysts of Table I, except that the indicated alumina/silica supports were treated with steam at an elevated temperature prior to impregnation with the molybdenum and nickel

compounds. In each case the steam-treated alumina/silica support was then impregnated with an aqueous solution of ammonium molybdate tetrahydrate, dried at 250° F. and then calcined for about 2 hours at 1000° F. The calcined composite was then impregnated with an aqueous solution of nickel acetate tetrahydrate, dried at about 250° F., followed by calcination for 2 hours at 1000° F. Each of these catalysts was then tested, using substantially the same test procedure employed in carrying out the previously described hydrogenation runs including preconditioning of the catalysts with a hydrogen stream containing 2 mole percent H<sub>2</sub>S at about 750° F. and about 325 p.s.i.g. for 1 hour. In each case benzene was used as the feed stock employing hydrogen containing 2 mole percent H<sub>2</sub>S as the carrier gas, and the hydrogenation was conducted at about 750° F. and about 320 to 325 p.s.i.g. at various flow rates of feed. The hydrogenation activity constant at 750° F. expressed as  $k_{750^{\circ} F}$ , was then calculated from the observed conversions. The results of these runs are given in the following Tables VI and VII, in which the results obtained with the corresponding catalyst prepared from the fresh "low" and "high" alumina/silica supports are also given for the purpose of comparison.

15  
TABLE VI

| Catalyst No.                                               | I    | III   | V    |
|------------------------------------------------------------|------|-------|------|
| Run No.                                                    | 25   | 26    | 27   |
| Composition:                                               |      |       |      |
| Percent MoO <sub>3</sub>                                   | 3.0  | 7.6   | 15.1 |
| Percent NiO                                                | 0.6  | 1.6   | 3.1  |
| Support                                                    | (1)  | (1)   | (1)  |
| Results: Hydrogenation activity constant $k_{750^\circ F}$ | 14   | 37.5  | 36   |
| Catalyst No.                                               | XIX  | XX    | XXI  |
| Run No.                                                    | 28   | 29    | 30   |
| Composition:                                               |      |       |      |
| Percent MoO <sub>3</sub>                                   | 3.0  | 7.6   | 15.1 |
| Percent NiO                                                | 0.6  | 1.6   | 3.1  |
| Support                                                    | (2)  | (2)   | (2)  |
| Results: Hydrogenation activity constant $k_{750^\circ F}$ | 17   | 37.5  | 44   |
| Catalyst No.                                               | XXII | XXIII | XXIV |
| Run No.                                                    | 31   | 32    | 33   |
| Composition:                                               |      |       |      |
| Percent MoO <sub>3</sub>                                   | 3.0  | 7.6   | 15.1 |
| Percent NiO                                                | 0.6  | 1.6   | 3.1  |
| Support                                                    | (3)  | (3)   | (3)  |
| Results: Hydrogenation activity constant $k_{750^\circ F}$ | 19   | 35    | 40   |

<sup>1</sup> Fresh 13% alumina/silica having a relative cracking activity of 1.5.

<sup>2</sup> 13% alumina/silica treated with 100% steam at atmospheric pressure for 24 hours at 1200° F. having a relative cracking activity of 0.6.

<sup>3</sup> 13% alumina/silica treated with 100% steam at atmospheric pressure for 24 hours at 1400° F. having a relative cracking activity of 0.3.

TABLE VII

| Catalyst No.                                               | IX     | X    | XI    |
|------------------------------------------------------------|--------|------|-------|
| Run No.                                                    | 34     | 35   | 36    |
| Composition:                                               |        |      |       |
| Percent MoO <sub>3</sub>                                   | 3.0    | 7.6  | 15.1  |
| Percent NiO <sub>3</sub>                                   | 0.6    | 1.6  | 3.1   |
| Support                                                    | (1)    | (1)  | (1)   |
| Results: Hydrogenation activity constant $k_{750^\circ F}$ | 22     | 46   | 65    |
| Catalyst No.                                               | XXV    | XXVI | XXVII |
| Run No.                                                    | 37     | 38   | 39    |
| Composition:                                               |        |      |       |
| Percent MoO <sub>3</sub>                                   | 3.0    | 7.6  | 15.1  |
| Percent NiO                                                | 0.6    | 1.6  | 3.1   |
| Support                                                    | (2)    | (2)  | (2)   |
| Results: Hydrogenation activity constant $k_{750^\circ F}$ | 25     | 51   | 48    |
| Catalyst No.                                               | XXVIII | XXIX | XXX   |
| Run No.                                                    | 40     | 41   | 42    |
| Composition:                                               |        |      |       |
| Percent MoO <sub>3</sub>                                   | 3.0    | 7.6  | 15.1  |
| Percent NiO                                                | 0.6    | 1.6  | 3.1   |
| Support                                                    | (3)    | (3)  | (3)   |
| Results: Hydrogenation activity constant $k_{750^\circ F}$ | 18     | 42   | 37    |

<sup>1</sup> Fresh 25% alumina/silica having a relative cracking activity of 1.5.

<sup>2</sup> 25% alumina/silica treated with 100% steam at atmospheric pressure for 24 hours at 1200° F. having a relative cracking activity of 0.5.

<sup>3</sup> 25% alumina/silica treated with 100% steam at atmospheric pressure for 24 hours at 1400° F. having a relative cracking activity of 0.3.

From the results of Table VI above it is apparent that steam treatment of the alumina/silica support containing 13 weight percent alumina prior to impregnation with the molybdenum and nickel compounds did not appreciably affect the hydrogenation activity of the catalysts. In fact, the activity of the catalysts containing about 3 and about

15 weight percent molybdenum oxide was increased by decreasing the relative cracking activity of the support; for example, compare the results of run numbers 25, 23 and 31 and of run numbers 27, 30 and 33. On the other hand, the results of Table VII demonstrate the fact that steam treatment at 1400° F. of the alumina/silica support containing 25 weight percent alumina appeared to have the effect of decreasing the hydrogenation activity especially at the higher level of molybdenum oxide concentration; for example, compare the results of runs 36, 39 and 42. Although the activity of Catalyst XXX, for example, was lower than Catalyst XI prepared from a fresh support, it still represents an improved hydrogenation catalyst. This is apparent by comparison of the results obtained with a catalyst supported on a different type of cracking support, namely silica/zirconia, such as Catalyst XXXI which was prepared as follows:

## CATALYST XXXI

To 20.45 grams of silica/zirconia, containing 20 weight percent silica which had been treated with 20 percent steam at 1200° F. for 17 hours, there was added a solution of 4.63 grams of ammonium molybdate tetrahydrate in 25 cc. of distilled water. The resultant paste was mixed thoroughly and then dried at 250° F. for 19 hours. The dried solid was ground to a powder and then calcined at 1000° F. for 2 hours. The calcined composite (23.8 grams) was then impregnated with a solution of 2.53 grams of nickel acetate tetrahydrate in 20 cc. of distilled water. The resultant paste was then dried at 250° F. for 20.5 hours, followed by calcination for 2 hours at 1000° F. The calculated composition, based upon ingredients, was 15.1 weight percent MoO<sub>3</sub>, 3.1 weight percent NiO, 16.4 weight percent ZrO<sub>2</sub> and 65.4 weight percent SiO<sub>2</sub>.

Catalyst XXXI was then tested for hydrogenation activity under substantially the same conditions as employed in the above-described hydrogenation runs. That is, 5.0 grams of Catalyst XXXI were charged to the above-described hydrogenation reactor and preconditioned with a hydrogen stream containing 2 mole percent H<sub>2</sub>S at 750° F., 325 p.s.i.g., for 1 hour. The hydrogen-hydrogen sulfide stream was then allowed to pick up benzene and the H<sub>2</sub>/H<sub>2</sub>S/benzene stream containing 0.55 mole percent benzene was then passed into the reactor at flow rates of 86, 123 and 181 standard cc. per minute at a reaction temperature of 750° F. and a pressure of 325 p.s.i.g. These flow rates yielded conversions of 40.8, 28.8 and 20.9, respectively, which corresponds to a hydrogenation activity constant, expressed as  $k_{750^\circ F}$ , of 8.8, which value is significantly lower than the value of the hydrogenation activity constants of the catalysts of this invention.

The following Catalysts XXXII to XXXIV were prepared to test the effect of preparational changes of hydrogenation activity. These catalysts were also tested for hydrogenation activity using benzene as the typical feed stock and using substantially the same test procedure described above. The specific operating conditions and results are set forth in the following Table VIII, in which the results obtained with Catalyst III above is also given for the purpose of comparison.

## CATALYST XXXII

To 68.18 grams of 13 percent alumina/silica there was added a solution of 6.96 grams of ammonium molybdate tetrahydrate in 75 cc. of distilled water. After thorough mixing, the paste was dried at 250° F. for 20.5 hours. The dried solid was then impregnated with a solution of 3.87 grams of nickel acetate tetrahydrate in 40 cc. of water. The mass was then stirred thoroughly, dried at 250° F. and then calcined for 2 hours at 1000° F. The calculated composition, based upon ingredients, is 7.55 weight percent MoO<sub>3</sub>, 1.55 weight percent NiO, 11.82 weight percent Al<sub>2</sub>O<sub>3</sub> and 79.07 weight percent SiO<sub>2</sub>.

This catalyst was prepared in the same manner as described for Catalyst XXXI, except that the final calcination step was effected for 2 hours at 1200° F. instead of 1000° F.

To 22.7 grams of freshly calcined silica/alumina containing 13 weight percent alumina, there was added an aqueous solution of 2.59 grams of phosphomolybdic acid ( $H_3PMo_{12}O_{40} \cdot xH_2O$ ) and 1.29 grams of nickel acetate tetrahydrate in 30 cc. of distilled water. The resultant paste was mixed thoroughly and was then dried at a temperature of 230° F. for about 18 hours, followed by calcination of 2 hours at 1000° F. The calculated composition, based upon ingredients, was 7.55 weight percent  $MoO_3$ , 1.55 weight percent  $NiO$ , 0.4 weight percent  $H_3PO_4$ , 68 weight percent  $SiO_2$  and 22.5 weight percent  $Al_2O_3$ .

Catalysts XXXII to XXXIV were tested using substantially the same test procedure as employed for testing the other catalysts. The operating conditions and results of these runs are tabulated in the following Table VIII.

the above-described catalysts in a laboratory hydrocracking test unit using alpha-methylnaphthalene as the typical test feed. In these tests, the reactor (8" long with 1/2" inner diameter) was charged with 2.5 to 10 grams of catalyst powder using glass wool as packing and alundum as the preheat zone. The reactor was connected into the unit and a hydrogen-hydrogen sulfide gas mixture containing 2 mole percent hydrogen sulfide was passed through the reactor at a pressure of from 780 to 800 pounds per square inch gage. The temperature was then raised to 900° F. and was held under these conditions for 1 or 2 hours while passing the hydrogen-hydrogen sulfide stream therethrough. At the start of each run, the hydrogen carrier gas was then allowed to mix with alpha-methylnaphthalene, in a mixing chamber at the inlet of the reactor. The alpha-methylnaphthalene was fed from a buret and Lapp pump. The products were passed out of the reactor through a water-cooled condenser into a high-pressure receiver maintained at 0° C. in which the liquid product was collected. The liquid product was weighed and distilled. Overhead, up to 400° F. vapor temperature, was taken as the gasoline product and the bottoms was considered cycle oil. Exit gas was expanded

TABLE VIII  
*Hydrogenation of benzene*

| Run No.                                                     | 43     |      | 44                 |      | 45                  |      | 46                 |      |
|-------------------------------------------------------------|--------|------|--------------------|------|---------------------|------|--------------------|------|
|                                                             | III    |      | XXXII <sup>1</sup> |      | XXXIII <sup>2</sup> |      | XXXIV <sup>3</sup> |      |
| <b>Composition:</b>                                         |        |      |                    |      |                     |      |                    |      |
| Percent $MoO_3$                                             | 7.6    |      | 7.6                |      | 7.6                 |      | 7.6                |      |
| Percent $NiO$                                               | 1.6    |      | 1.6                |      | 1.6                 |      | 1.6                |      |
| Support                                                     | (4)    |      | (4)                |      | (4)                 |      | (4)                |      |
| <b>Pretreatment of Catalyst:</b>                            |        |      |                    |      |                     |      |                    |      |
| Catalyst charge, grams                                      | 1.0    |      | 1.0                |      | 1.0                 |      | 1.0                |      |
| Catalyst Temperature, ° F.                                  | 750    |      | 750                |      | 750                 |      | 750                |      |
| Reaction Pressure, p.s.i.g.                                 | 325    |      | 325                |      | 325                 |      | 325                |      |
| Gas Composition                                             | (5)    |      | (5)                |      | (5)                 |      | (5)                |      |
| Treatment time, hours                                       | 1.0    |      | 1.0                |      | 1.0                 |      | 1.0                |      |
| <b>Test Conditions:</b>                                     |        |      |                    |      |                     |      |                    |      |
| Catalyst Temperature, ° F.                                  | 750    |      | 750                |      | 750                 |      | 750                |      |
| Reaction Pressure, p.s.i.g.                                 | 325    |      | 325                |      | 325                 |      | 325                |      |
| Flow rate, standard cc./min.                                | 132    | 82   | 143                | 100  | 106                 | 230  | 107                | 152  |
| Feed                                                        | (6)    | (6)  | (6)                | (6)  | (6)                 | (6)  | (6)                | (6)  |
| Carrier Gas                                                 | (3)    | (3)  | (3)                | (3)  | (3)                 | (3)  | (3)                | (3)  |
| <b>Results:</b>                                             |        |      |                    |      |                     |      |                    |      |
| Conversion, percent                                         | 24.6   | 31.8 | 13.5               | 34.0 | 22.0                | 15.9 | 30.3               | 27.3 |
| Hydrogenation activity constant $k_{750^{\circ} F}$         | 37.5   |      | 37.5               |      | 43.7                |      | 40.2               | 29.2 |
| Space velocity required to obtain 90% conversion of benzene | 0.0089 |      | 0.0089             |      | 0.0104              |      | 0.0133             |      |

<sup>1</sup> The silica/alumina support impregnated with ammonium molybdate was not calcined prior to impregnation with nickel acetate.

<sup>2</sup> The silica/alumina support impregnated with ammonium molybdate was not calcined prior to impregnation with nickel acetate and the final calcination temperature was 1200° F.

<sup>3</sup> The catalyst was prepared by co-impregnation of the silica/alumina support with phosphomolybdic acid and nickel acetate.

<sup>4</sup> 13% alumina/silica.

<sup>5</sup> 2 mole percent  $H_2S$  in  $H_2$ .

<sup>6</sup> Benzene.

From the results of Table VIII above it is apparent that omission of the calcination step between the ammonium molybdate and nickel acetate impregnations yielded a catalyst, i.e. Catalyst XXXII, equivalent in activity to Catalyst III, in which the ammonium molybdate impregnated alumina/silica support was calcined prior to the addition of the nickel acetate solution. However, a final calcination of the catalyst at 1200° F. as in Catalyst XXXII, improved catalyst activity about 15 percent; for example, compare the results of run numbers 44 and 45. As apparent from run number 46, co-impregnation of the alumina/silica support with a solution of phosphomolybdic acid and nickel acetate improved the activity of the catalyst markedly, i.e. from a hydrogenation activity ( $k_{750^{\circ} F}$ ) of 37.5 to 56.

The relative effectiveness of the catalysts of this invention as hydrocracking catalysts was determined by using

through a regulator into a low temperature glass receiver maintained at -60° C. and was metered. Product gas was analyzed by mass spectrometry. The amount of carbon laydown on the catalyst was determined by combustion. Refractive index of the gasoline and cycle oil was used as a measure of the amount of hydrogenation. In these tests, the above described Catalysts I-III, VIII-XI, XX-XXVI, XXXIII and XXXIV were employed. For the purpose of comparison, a commercially available cobalt molybdate catalyst analyzing 13.8 weight percent  $MoO_3$ , 3.1 weight percent  $CoO$ , 0.9 weight percent  $SiO_2$  and 82.2 weight percent  $Al_2O_3$  also was tested under substantially the same operating conditions; this latter catalyst is designated as Catalyst XXXV. The specific operating conditions and results obtained in testing the catalysts of this invention as hydrocracking catalysts, are set forth in the following Table IX.

19  
TABLE IX  
*Hydrocracking tests*

| Run No.                                                         | 1     | 2     | 3     | 4     | 5     | 6      | 5  |
|-----------------------------------------------------------------|-------|-------|-------|-------|-------|--------|----|
| Catalyst No.                                                    | I     | IX    | II    | III   | XX    | XXXIII | 10 |
| Composition:                                                    |       |       |       |       |       |        |    |
| Percent MoO <sub>3</sub>                                        | 3.0   | 3.0   | 6.0   | 7.6   | 7.6   | 7.6    |    |
| Percent NiO                                                     | 0.6   | 0.6   | 1.2   | 1.6   | 1.6   | 1.6    |    |
| Alumina/Silica Support,                                         |       |       |       |       |       |        |    |
| Weight Percent Alumina                                          | 13    | 25    | 13    | 13    | 13    | 213    |    |
| Weight, grams                                                   | 10    | 5     | 10    | 5.0   | 5.0   | 2.5    |    |
| Activation, 2 Mole Percent H <sub>2</sub> S in H <sub>2</sub> : |       |       |       |       |       |        |    |
| Temperature, °F                                                 | 900   | 900   | 900   | 900   | 900   | 900    |    |
| Pressure, p.s.i.g.                                              | 780   | 800   | 800   | 800   | 800   | 800    |    |
| Time, hours                                                     | 1.25  | 1     | 2     | 1.0   | 1.0   | 1      | 15 |
| Gas rate, cu. ft./hr.                                           |       |       |       |       |       |        |    |
| 70° F                                                           | 0.592 | 0.502 | 0.615 | 0.505 | 0.635 | 0.530  |    |
| Operating conditions:                                           |       |       |       |       |       |        |    |
| Temperature, °F                                                 | 900   | 900   | 900   | 900   | 900   | 900    |    |
| Pressure, p.s.i.g.                                              | 750   | 800   | 860   | 800   | 774   | 890    |    |
| Time, hours                                                     | 2     | 2     | 2     | 2     | 2     | 2      |    |
| Space velocity, w./hr./w.                                       | 1.14  | 4.25  | 1.04  | 2.13  | 2.07  | 3.9    |    |
| Gas/Oil, M./M.                                                  | 8.2   | 5.0   | 9.9   | 9.8   | 19.1  | 11.3   | 20 |
| Yields, Weight Percent                                          |       |       |       |       |       |        |    |
| Output:                                                         |       |       |       |       |       |        |    |
| Gas (C <sub>1</sub> -C <sub>4</sub> )                           | 13.6  | 2.4   | 13.8  | 7.7   | 4.6   | 5.0    |    |
| Gasoline                                                        | 42.3  | 21.0  | 53.5  | 62.5  | 47.3  | 35.6   |    |
| Cycle Oil                                                       | 36.6  | 75.5  | 28.9  | 38.0  | 47.2  | 58.8   |    |
| Carbon                                                          | 7.5   | 1.1   | 4.3   | 1.8   | 0.9   | 0.6    |    |
| Conversion, Weight Percent (single pass)                        | 63.4  | 24.5  | 71.1  | 62.0  | 52.8  | 41.2   | 25 |
| Product Inspections:                                            |       |       |       |       |       |        |    |
| Δn <sup>20</sup> p (Feed minus Gasoline) × 10 <sup>4</sup>      | 1,272 | 1,216 | 1,477 | 1,287 | 1,233 | 1,135  |    |
| Δn <sup>20</sup> p (Feed minus Cyclo Oil) × 10 <sup>4</sup>     | 160   | 268   | 307   | 253   | 319   | 254    |    |
| Relative Hydrocracking Activity                                 | 0.6   | 0.5   | 0.7   | 1.0   | 0.4   | 0.9    | 30 |
| Carbon Producing Factor                                         | 3.8   | 3.9   | 1.6   | 1.0   | 2.4   | 0.9    |    |
| Hydrogenation Activity Constant, k <sub>750</sub> ° F           | 14    | 22    | 18    | 37.5  | 38    | 44     |    |

| Run No.                                                         | 7     | 8     | 9     | 10    | 11    | 12    | 35 |
|-----------------------------------------------------------------|-------|-------|-------|-------|-------|-------|----|
| Catalyst No.                                                    | XXXIV | X     | XXVI  | XI    | VIII  | XXXV  |    |
| Composition:                                                    |       |       |       |       |       |       |    |
| Percent MoO <sub>3</sub>                                        | 7.6   | 7.6   | 7.6   | 15.1  | 30.0  | 13.8  |    |
| Percent NiO                                                     | 1.6   | 1.6   | 1.6   | 3.1   | 6.3   | (4)   |    |
| Alumina/Silica Support, Weight Percent Alumina                  | 13    | 25    | 125   | 25    | 13    | (6)   | 40 |
| Weight, grams                                                   | 5     | 5     | 5     | 5     | 5     | 10    |    |
| Activation, 2 Mole Percent H <sub>2</sub> S in H <sub>2</sub> : |       |       |       |       |       |       |    |
| Temperature, °F                                                 | 900   | 900   | 900   | 900   | 900   | 900   |    |
| Pressure, p.s.i.g.                                              | 800   | 800   | 800   | 800   | 800   | 800   |    |
| Time, hours                                                     | 1     | 1     | 1     | 1     | 1     | 1     | 45 |
| Gas rate, cu. ft./hr.                                           |       |       |       |       |       |       |    |
| 70° F                                                           | 0.632 | 0.545 | 0.521 | 0.531 | 0.620 | 0.455 |    |
| Operating Conditions:                                           |       |       |       |       |       |       |    |
| Temperature, °F                                                 | 900   | 900   | 900   | 900   | 900   | 900   |    |
| Pressure, p.s.i.g.                                              | 800   | 787   | 800   | 890   | 800   | 800   |    |
| Time, hours                                                     | 2     | 2     | 2     | 2     | 2     | 2     |    |
| Space velocity, w./hr./w.                                       | 4.02  | 4.14  | 4.07  | 4.07  | 2.10  | 1.12  | 50 |
| Gas/Oil, M./M.                                                  | 4.97  | 5.2   | 4.83  | 5.0   | 9.6   | 10.4  |    |
| Yields, Weight Percent                                          |       |       |       |       |       |       |    |
| Output:                                                         |       |       |       |       |       |       |    |
| Gas (C <sub>1</sub> -C <sub>4</sub> )                           | 3.7   | 2.4   | 3.2   | 2.8   | 2.2   | 1.8   |    |
| Gasoline                                                        | 25.0  | 24.5  | 18.4  | 12.7  | 21.4  | 10.3  |    |
| Cycle Oil                                                       | 67.8  | 71.9  | 76.3  | 82.1  | 75.0  | 86.7  |    |
| Carbon                                                          | 3.5   | 1.2   | 2.1   | 2.4   | 1.4   | 1.2   | 55 |
| Conversion, Weight Percent (single pass)                        | 32.2  | 28.1  | 23.7  | 17.9  | 25.0  | 13.3  |    |
| Product Inspections:                                            |       |       |       |       |       |       |    |
| Δn <sup>20</sup> p (Feed minus Gasoline) × 10 <sup>4</sup>      | 1,208 | 1,188 | 1,174 | 1,331 | 1,172 | 1,083 |    |
| Δn <sup>20</sup> p (Feed minus Cycle Oil) × 10 <sup>4</sup>     | 278   | 288   | 278   | 311   | 342   | 267   | 60 |
| Relative Hydrocracking Activity                                 | 1.5   | 0.6   | 0.9   | 0.7   | 0.3   | 0.08  |    |
| Carbon Producing Factor                                         | 1.4   | 3.5   | 1.3   | 1.9   | 5.2   | 12    |    |
| Hydrogenation Activity Constant, k <sub>750</sub> ° F           | 56    | 46    | 51    | 65    | 20    | 4.4   |    |

<sup>1</sup> Alumina/silica support treated with 100% steam at atmospheric pressure for 24 hours to a relative cracking activity of 0.5.

<sup>2</sup> The alumina/silica support impregnated with ammonium molybdate was not calcined prior to impregnation with nickel acetate and the final calcination temperature was 1200° F.

<sup>3</sup> The catalyst was prepared by co-impregnation of the silica/alumina support with phosphomolybdc acid and nickel acetate.

<sup>4</sup> 3.1% CoO.

<sup>5</sup> 0.9% SiO<sub>2</sub>/82.2% Al<sub>2</sub>O<sub>3</sub>.

The low hydrocracking activity and poor selectivity of the cobalt molybdate catalyst, i.e. Catalyst XXXV employed in run No. 12 of Table IX necessitated the adoption of the more active Catalyst III employed in run number 4 as the reference catalyst. The relative hydro-

cracking activity values set out in Table IX are defined as the space velocity of the particular run divided by the space velocity at the same conversion level obtained with Catalyst III. The carbon producing factor is defined as the carbon yield obtained in the particular run divided by the carbon yield for Catalyst III at the same conversion level.

From the results of Table IX, it is apparent that an improved hydrocracking process is obtained by the use of the catalysts of the present invention which catalysts also possess high hydrogenation activity. For example, the hydrogenation activity of Catalyst XXXV employed in run No. 12 was one-third that of Catalyst I and only about one-fifteenth as active as Catalyst III. Notwithstanding the fact that the hydrocracking activity of Catalyst XXXV was low, its tendency to produce carbon was excessive; for example, compare the carbon producing factor of 12 exhibited by Catalyst XXXV with the carbon producing factor of 1.0 obtained with Catalyst III. Thus, from the standpoint of catalyst life and yields of desired liquid product, a catalyst such as typically represented by Catalyst XXXV which possesses high tendency to produce carbon is undesirable for use in a hydrocracking process.

Although catalysts prepared from alumina/silica containing 25 weight percent alumina, such as Catalyst X, employed in run No. 8, exhibited relatively less hydrocracking activity and a somewhat greater tendency to produce carbon than the catalysts prepared from the "low" alumina/silica support, it is to be noted that steam treatment of the 25 weight percent alumina/silica support greatly enhanced the activity of the catalyst and significantly increased its selectivity as evidenced by a lowering of the carbon producing factor; for example, compare the results obtained in run No. 9, which employed the steam treated Catalyst XXVI with those employed in run No. 8, prepared from the fresh 25 weight percent alumina/silica support. In this connection it is to be further noted that a similar steam treatment of the 13 weight percent alumina/silica support tended to yield a catalyst of lower hydrocracking activity and selectivity than one prepared from the same support which was not steam treated; for example, compare the results obtained in run No. 5 which employed Catalyst XX prepared from the steam treated support with run No. 4 which employed Catalyst III prepared from the fresh support.

As noted above, co-impregnation of the silica/alumina support with phosphomolybdc acid and nickel acetate yielded a catalyst of improved hydrogenation activity as compared with one in which the support was impregnated successively with the respective precursors of the molybdenum and nickel catalytic agents. In regard to hydrocracking activity, the same increase in activity was also observed. This is demonstrated, for example, by comparing the relative hydrocracking activity (1.5) of Catalyst XXXIV employed in run number 7 of Table IX with the relative hydrocracking activity (1.0) observed with Catalyst III employed in run number 4.

Further improvement in the hydrocracking activity of the catalysts of this invention is realized by incorporating therein a minor proportion of a compound of cobalt in an amount between about 0.2 and about 2.0 weight percent based on the total weight of the catalyst. Such catalysts are typically represented by Catalyst XXXVI which was prepared as follows:

#### CATALYST XXXVI

To 22.53 grams of silica/alumina containing 13 weight percent alumina, there was added an aqueous solution of 2.3 grams of ammonium molybdate tetrahydrate in 35 cc. of distilled water. The resultant paste was mixed thoroughly, excess water was evaporated, and was then dried in an oven at 250° F. for about 22.5 hours. The dried solid was then ground to a powder and calcined for 2 hours at 1000° F. The calcined composite (23.17 grams) was then impregnated with a solution containing

1.2 grams of nickel acetate tetrahydrate and 0.72 gram of cobalt nitrate hexahydrate in 25 cc. of distilled water. The resultant paste was then mixed thoroughly while excess water was evaporated and was dried in an oven at 250° F. for about 22 hours. The dried solid was then ground to a powder and calcined for 2 hours at 1000° F. The calculated composition, based upon ingredients added, was 7.55 weight percent MoO<sub>3</sub>, 1.55 weight percent NiO, 0.79 weight percent CoO, 78.4 weight percent SiO<sub>2</sub> and 11.7 weight percent Al<sub>2</sub>O<sub>3</sub>.

The hydrocracking activity and selectivity of Catalyst XXXVI was tested as described above for effecting the hydrocracking tests of Table IX using alpha-methylnaphthalene as the feed and the above-described hydrocracking test procedure. The specific operating conditions employed are set forth in the following Table X, which also sets forth the results obtained with the above-described Catalyst III, which did not contain the cobalt oxide promoter.

TABLE X  
*Hydrocracking of alpha-methyl naphthalene*

| Run No.                                                               | 13    | 14    |
|-----------------------------------------------------------------------|-------|-------|
| Catalyst No.                                                          | XXXVI | III   |
| <b>Composition:</b>                                                   |       |       |
| Percent MoO <sub>3</sub>                                              | 7.6   | 7.6   |
| Percent NiO                                                           | 1.6   | 1.6   |
| Percent CoO                                                           | 0.8   | 0     |
| Support                                                               | (1)   | (1)   |
| Weight, grams                                                         | 5.0   | 5.0   |
| Activation, 2 Mole Percent H <sub>2</sub> S in H <sub>2</sub> :       |       |       |
| Temperature, ° F                                                      | 900   | 900   |
| Pressure, p.s.i.g.                                                    | 800   | 800   |
| Time, hours                                                           | 1     | 1     |
| Gas, rate, cu. ft./hr. 70° F                                          | 0.535 | 0.505 |
| Operating Conditions:                                                 |       |       |
| Temperature, ° F                                                      | 900   | 900   |
| Pressure, p.s.i.g.                                                    | 800   | 800   |
| Time, hours                                                           | 2     | 2     |
| Space velocity, w./hr./w.                                             | 3.65  | 2.13  |
| Gas/Oil, M./M.                                                        | 5.88  | 9.8   |
| Yields, Weight Percent Output:                                        |       |       |
| Gas (C <sub>1</sub> -C <sub>4</sub> )                                 | 4.1   | 7.7   |
| Gasoline                                                              | 28.1  | 52.5  |
| Cycle Oil                                                             | 65.2  | 38.0  |
| Carbon                                                                | 2.6   | 1.8   |
| Conversion, Weight Percent (single pass)                              | 34.8  | 62.0  |
| Product Inspections:                                                  |       |       |
| Δn <sub>D<sup>20</sup></sub> (Feed minus Gasoline) × 10 <sup>4</sup>  | 1,191 | 1,287 |
| Δn <sub>D<sup>20</sup></sub> (Feed minus Cycle Oil) × 10 <sup>4</sup> | 259   | 233   |
| Relative Hydrocracking Activity                                       | 1.5   | 1.0   |
| Carbon Producing Factor                                               | 1.0   | 1.0   |

<sup>1</sup> 13 weight percent alumina/silica.

From the results of Table X, it is apparent that incorporation of a minor proportion of a promoter comprising a compound of cobalt increased the relative hydrocracking activity from 1.0 to 1.5 or increased the hydrocracking activity of the catalyst by 50 percent. It is to be further noted that this improvement in hydrocracking activity was obtained without any adverse effect on the carbon producing factor.

In order to compare the hydrocracking activity of the catalysts of this invention with another type of catalyst comprising catalytic agents of molybdenum and nickel on a different commercial cracking catalyst, the following Catalysts XXXVII and XXXVIII were tested, the support used being a commercial silica/magnesia cracking catalyst containing 30 weight percent magnesia based on the weight of the support.

#### CATALYST XXXVII

To 45.45 grams of commercial magnesia/silica cracking catalyst containing 30 weight percent magnesia, there was added a solution of 4.6 grams of ammonium molybdate tetrahydrate in 40 cc. of distilled water. After mixing thoroughly, the paste was dried at 250° F. for 24 hours and was then calcined for 2 hours at 1000° F. To the calcined composite (45.72 grams), there was added a solution of 2.3 grams of nickel acetate tetrahydrate in 45 cc. of distilled water. Excess water was then evaporated, the mixture was mixed thoroughly and was then

dried at 250° F. for about 24.5 hours followed by calcination for 2 hours at 1000° F. The calculated composition of the final catalyst, based upon ingredients, was 7.55 weight percent MoO<sub>3</sub>, 1.55 weight percent NiO, 27.5 weight percent MgO, and 63 weight percent SiO<sub>2</sub>.

#### CATALYST XXXVIII

To 40.9 grams of commercial magnesia/silica cracking catalyst containing 30 weight percent magnesia, there was added a solution of 9.26 grams of ammonium molybdate tetrahydrate in 40 cc. of distilled water. After mixing thoroughly, the paste was dried at 250° F. for 22 hours, followed by calcination for 2 hours at 1000° F. To the calcined composite (45.8 grams), there was added a solution of 4.8 grams of nickel acetate tetrahydrate in 45 cc. of distilled water. Excess water was evaporated, and the mixture was then dried in an oven at 250° F. followed by calcination for 2 hours at 1000° F. The calculated composition, based upon ingredients, was 15.10 weight percent MoO<sub>3</sub>, 3.10 weight percent NiO, 24 weight percent MgO and 57 weight percent SiO<sub>2</sub>.

The silica/magnesia supported Catalysts XXXVII and XXXVIII were tested for hydrocracking activity and selectivity as described above for effecting the hydrocracking runs of Table IX, using alpha-methylnaphthalene as the feed and substantially the same test procedure. The specific operating conditions employed in these runs and results are tabulated in the following Table XI.

TABLE XI  
*Hydrocracking of alpha-methyl naphthalene*

| Run No.                                                               | 15     | 16      |
|-----------------------------------------------------------------------|--------|---------|
| Catalyst No.                                                          | XXXVII | XXXVIII |
| <b>Composition:</b>                                                   |        |         |
| Percent MoO <sub>3</sub>                                              | 7.6    | 15.1    |
| Percent NiO <sub>3</sub>                                              | 1.6    | 3.1     |
| Support                                                               | (1)    | (1)     |
| Weight, grams                                                         | 10     | 10      |
| Activation, 2 Mole Percent H <sub>2</sub> S in H <sub>2</sub> :       |        |         |
| Temperature, ° F                                                      | 900    | 900     |
| Pressure, p.s.i.g.                                                    | 800    | 800     |
| Time, hours                                                           | 1.66   | 1.23    |
| Gas rate, cu. ft./hr. 70° F                                           | 0.678  | 0.663   |
| Operating Conditions:                                                 |        |         |
| Temperature, ° F                                                      | 900    | 900     |
| Pressure, p.s.i.g.                                                    | 800    | 800     |
| Time, hours                                                           | 2      | 2       |
| Space velocity, w./hr./w.                                             | 1.03   | 1.07    |
| Gas/Oil, M./M.                                                        | 10.0   | 9.5     |
| Yields, Weight Percent Output:                                        |        |         |
| Gas (C <sub>1</sub> -C <sub>4</sub> )                                 | 4.2    | 4.9     |
| Gasoline                                                              | 13.9   | 20.9    |
| Cycle Oil                                                             | 79.0   | 70.8    |
| Carbon                                                                | 2.9    | 3.4     |
| Conversion, Weight Percent (single pass)                              | 21.0   | 29.2    |
| Product Inspections:                                                  |        |         |
| Δn <sub>D<sup>20</sup></sub> (Feed minus Gasoline) × 10 <sup>4</sup>  | 1,043  | 1,111   |
| Δn <sub>D<sup>20</sup></sub> (Feed minus Cycle Oil) × 10 <sup>4</sup> | 166    | 146     |
| Relative Hydrocracking Activity                                       | 0.1    | 0.2     |
| Carbon Producing Factor                                               | 14     | 9       |

<sup>1</sup> 30 weight percent magnesia/silica.

Inspection of the results obtained in runs 15 and 16 of Table XI in which the silica/magnesia supported catalysts were employed shows that these catalysts possessed a significantly lower hydrocracking activity as compared with the catalysts of this invention and, in addition, exhibited a severe tendency to produce carbon, the carbon producing factors of these particular catalysts being of the same order as observed with the above cobalt/molybdate Catalyst XXXV employed in run number 12 of Table IX above.

From the above, it is apparent that the catalyst of this invention possess a particularly good combination of hydrogenation and cracking activity which renders them particularly useful for converting residual hydrocarbon oils, tars, waxes and other heavy materials remaining after lighter fractions such as those boiling within the gasoline boiling range have been removed from refinery process streams, to lower boiling and more useful hydrocarbon fractions. Because of their high hydrogenation activity, the products such as gasoline boiling range prod-

23

uct, possess only a low degree olefinic unsaturation and thus do not necessarily have to be submitted to further hydrogenation before use.

When used as hydrocracking catalysts, the superior catalysts of this invention, are those containing from about 6 to about 20 weight per cent of the compound of molybdenum, the compound of nickel being present in an amount to provide an atom ratio of molybdenum to nickel of between about 1 and about 3, particularly between about 2 and about 3. When a low alumina/silica cracking base is employed, particularly active and selective catalysts are those containing the compound of molybdenum in an amount between about 6 and about 12 weight percent. When a high alumina/silica cracking base is employed, the superior catalysts are those containing from about 10 to about 20 weight percent of the compound of molybdenum; or catalysts in which the content of molybdenum compound ranges between about 6 and about 10 weight percent and in which the high alumina/silica support has been treated with steam at an elevated temperature such as between about 600° F. and about 1250° F. for a period of time between about 0.5 and about 48 hours.

Due to their low carbon producing tendency, the catalysts of this invention may be used for long periods of time without requiring regeneration or reactivation. However, after the catalysts have become deactivated due to prolonged use, they may be regenerated by treatment with hydrogen at an elevated temperature to remove sulfur as hydrogen sulfide followed by treatment with oxygen or an oxygen-containing gas to burn off carbon, and then subjected to treatment with a hydrogen-hydrogen sulfide stream under the aforesaid conditions.

24

Various alterations and modifications of the hydrogenerative processes, catalysts and methods of preparing the catalysts of this invention may become apparent to those skilled in the art without departing from the scope of this invention.

Having described our invention, we claim:

A process for the destructive hydrogenation of a hydrocarbon fraction boiling above the gasoline boiling range which comprises treating a catalyst comprising nickel oxide and between about 6 and about 20 weight percent of molybdenum oxide, and between about 0.2 and about 2 weight percent of cobalt oxide supported on a silica/alumina carrier containing between about 10 and about 30 weight percent alumina, the atom ratio of molybdenum to nickel being between about 1 and about 3, with hydrogen sulfide at an elevated temperature, and contacting said hydrocarbon fraction with said catalyst in the presence of a hydrogen-rich gas at a temperature between about 600° F. and about 925° F. such that conversion of said hydrocarbon fraction to lower boiling normally liquid product is effected.

References Cited in the file of this patent

UNITED STATES PATENTS

|           |                |               |
|-----------|----------------|---------------|
| 2,758,957 | Nozaki         | Aug. 14, 1956 |
| 2,799,626 | Johnson et al. | July 16, 1957 |
| 2,888,397 | Burton et al.  | May 26, 1959  |
| 2,917,448 | Beuther et al. | Dec. 15, 1959 |
| 2,944,961 | McAfee         | July 12, 1960 |
| 2,951,807 | Kirberg        | Sept. 6, 1960 |